

Feb. 2, 1965

D. R. ADAMS

3,168,387

ABRASIVES

Filed Nov. 17, 1959



Fig. 1.



Fig. 2.



Fig. 3.



Fig. 4.

INVENTOR.

Donald R. Adams

BY

*Delmar H. Jensen*

Agent.

# United States Patent Office

3,168,387

Patented Feb. 2, 1965

1

3,168,387

ABRASIVES

Donald R. Adams, Santa Monica, Calif.  
(9000 Sunset Blvd., Suite 319, Los Angeles, Calif.)  
Filed Nov. 17, 1959, Ser. No. 853,582  
31 Claims. (Cl. 51—295)

This invention relates to abrasives, and more particularly to improvements in abrasive articles of the type made from a plurality of abrasive granules, such as coated abrasive papers, grinding wheels and the like.

Abrasive articles made by bonding a large number of relatively small granules of solid abrasive materials, either to a backing such as a paper, fiber, cloth or metal sheet, or formed into a coherent mass such as a grinding wheel or block or a cutting wheel, are extremely common in industry and even household use.

In spite of much research and development effort which has gone into the articles of this type, these abrasives are not always perfect, and suffer from a number of disadvantages. For example, in the case of grinding wheels more abrasive particles are consumed than actually go into the grinding or cutting operation itself; otherwise stated, the grinding efficiency is far from 100% considering the potential abrasive material present. This comes about as a result of chipping of individual abrasive granules, as well as the dislodgement of abrasive granules from the matrix in which they are contained before they have been consumed by normal grinding. The same difficulties appear in coated abrasives such as emery cloth, sand paper, and the like, and indeed generally to an even higher degree. Commonly, the abrasive granule layer on coated abrasives is only one particle thick, and long before individual particles are worn down to even half of their original size, they are often dislodged from their bond to the backing, or the backing itself becomes partially destroyed or damaged in portions of the sheet material so that it must be discarded. Another disadvantage common to the abrasive materials described is that they are all subject to maximum limits of grinding speed. As attempts are made to grind faster than a maximum rate which depends upon the particular abrasive article used and the material being ground or abraded, then over-heating rapidly leads to an excessive rate of consumption or even destruction of the abrasive article. Maximum grinding rates can be increased by wet grinding as distinguished from dry grinding, wherein a coolant fluid is used, such as water, but even in these cases localized heating at the actual cutting surface of the abrasive granule sets an upper limit to grinding speeds.

It is an object of this invention to increase the durability of abrasive articles.

Another object of the invention is to provide a method for increasing the maximum grinding speed for a given abrasive article.

Another object of the invention is to provide abrasive articles which develop less frictional heat when used in a grinding process.

A further object of the invention is to provide abrasive articles having enhanced heat dissipating properties.

Another object of the invention is to provide an abrasive article which exhibits decreased consumption of abrasive material when in use, while yet maintaining efficient grinding action.

Other objects of the invention will appear as the description thereof proceeds.

Generally speaking, and in accordance with an illustrative embodiment of the invention, the objects thereof are accomplished by providing a relatively thin adherent coating containing a metal-leaf pigment, as hereafter defined, on the exposed surfaces of abrasive granules contained either as a coating on a sheet or other substratum, or

2

contained in a coherent mass as in a grinding wheel, the coating likewise being applied to any bonding material serving to hold the individual abrasive granules in place.

A description of the invention will be facilitated by reference to the drawings, in which:

FIGURE 1 is a cross-section of an abrasive article of the so-called "coated" type.

FIGURE 2 is a cross-section of a coated abrasive article as in FIGURE 1, after use.

FIGURE 3 is a cross-section of a portion of an abrasive article of the coherent type such as a grinding wheel, after use.

FIGURE 4 is a sectional view of a coated abrasive with a backing layer to be described.

The abrasive particles, such as indicated by reference characters 10 and 30 in FIGURES 1, 2 and 3, are commonly flint, garnet, alumina, silicon carbide, crushed glass, crushed quartz, or the like. For sandpapers, the relatively cheap flint and garnet are widely used, while in grinding wheels, the better types of coated abrasive cloth, and the like, alumina, tungsten carbide, and silicon carbide may be used. Crushed diamonds may also be used, as well as boron carbide. My invention is applicable to all such abrasives, including but not limited to those specifically mentioned. The form of the abrasive particle is almost always substantially isodimensional, that is, the abrasive particles are neither flakes nor fibers, but the individual particles have dimensions in all three coordinates of about the same order of magnitude for a given particle, even though some of the particles may be somewhat elongated. The actual size of the particles varies considerably depending upon the abrasive article desired and the type of service contemplated. In general, abrasive sizes in common use range from about 10 mesh to about 200 mesh and finer. Again, my invention is applicable regardless of size, as may be seen from the latter description herein.

In order for the abrasive particles to abrade the objects to be ground or otherwise worked on, it is necessary to hold the abrasive particles in place. This is accomplished by means of a bonding agent. Those in common use are quite diverse, ranging from hide and starch glues for cheaper types of sandpaper, through other organic adhesives such as varnish-type vehicles, shellac, alkyd resins, various phenolic resins, polyester adhesives, natural and synthetic rubber adhesives and various other synthetic plastics, to inorganic bonding agents such as sodium silicate, other silicates, ceramic bodies and the like. In some cases the abrasive particles may be made to cohere by raising the temperature of a compressed mass of particles until sintering takes place. In this case, the abrasive particle itself becomes its own bond, and in this description and in the claims which follow, the term "bonding material" or "bonding agent" will be understood to include the abrasive material itself when caused to act in this manner. The very hardest abrasives, however, tend to have very high melting points, so that it is more common to use a bonding agent other than the abrasive particle material itself. Where a sheet or plate of metal is used as a support for the abrasive granules, the latter can of course be attached by any of the adhesives already mentioned, and may even be brazed to the metal with another metal or metallic alloy of lower melting point. Thus, silicon carbide granules may be brazed with copper to a steel sheet.

The abrasive particles may be bonded to a suitable backing, or they may be bonded to themselves. In the specific embodiment shown in FIGURE 1, the abrasive particles 10 may be for example silicon carbide, while the backing sheet 11 may be any suitable paper, cloth, fiber, metal or like sheet, most generally solid, but sometimes in mesh form. It may be noted that paper and

cloth are the commonest backing materials, and are generally heavily treated with various sizing coats so as to possess flexibility, toughness, and in some cases resistance to water, and also so as to present a suitable surface to which the abrasive particles may be bonded. It is not necessary to describe the various treatments commonly applied to sheet backing materials in view of the fact that these are well-known to the art and that my invention is applicable to all coated abrasives regardless of the nature of the backing material.

Where the abrasive particles are coated on to a sheet material, the bonding agent generally forms a layer on the coated side immediately adjacent to and adherent to the backing material. Such a layer of bonding material is indicated by reference character 12 in FIGURE 1. The abrasive particles 10 are firmly embedded in and held by the bonding material 12. This is generally accomplished by applying the abrasive particles to the bonding material while it is still in a fluid or semi-fluid, sticky condition, and moreover by applying one or more light coats of additional bonding or sizing material, generally in a suitable solvent, or in some cases merely a coating of bonding material solvent itself, to the coated abrasive so that the bonding agent tends to grip at least a portion of the sides of the abrasive particles as well as those portions in substantially direct contact with the backing material. This condition is clearly evident in FIGURE 1, where a thin layer of bonding material is shown on most of the particles, for example, at the point indicated by 13, but may be absent from the generally exposed portions of some of the grains, as in the particle indicated by reference character 14 in FIGURE 1. It is immaterial for the practice of my invention whether the abrasive particles are exposed completely over some of their surface or are fairly well covered by a thin coating of bonding material.

Where the abrasive article is a coherent mass of particles, as for example in the case of an abrasive wheel, an abrasive block or whetstone, or the like, the bonding material generally joins the portions of the particles which are in actual or approximate contact, with void space generally left in between the particles. The situation in most abrasive articles of this type is quite analogous to a mass of sand with a relatively small amount of water, wherein the water is present at the points of contact of the sand particles but not elsewhere. In fact, the circumstance that the bonding agent is generally in a liquid or semi-liquid form at some stage of the manufacture causes it to assume the same position that water does in a mass of sand and indeed for the same reason, i.e. capillarity. In FIGURE 3, the void spaces 33 appear between the particles, which in turn are joined by bonding material 32.

It should be noted that FIGURES 1, 2, 3 and 4 are not only sections, they are indeed thin sections or slices through the articles in question, this having been done for clarity of presentation.

As mentioned, in accordance with my invention, the exposed portions of the abrasive particles, together with any exposed portions of bonding agent, in abrasives of the types described, are coated with a thin layer of a metal pigment, and more particularly a metal-leaf pigment, in a suitable vehicle.

A wide variety of metals may be used, although I prefer those that have corrosion resistance and in general some ductility. Hardness is not especially necessary or desired, and indeed relatively soft metals are very useful, although readily fusible metals are not desirable. Suitable metals include aluminum; aluminum alloys, especially with beryllium; copper; a wide variety of copper alloys including copper-zinc, copper lead and copper-zinc-lead alloys, thus including the various brasses and bronzes; beryllium copper; stainless steel; nickel; nickel alloys; gold; silver; the platinum metals; and the like.

The metal-leaf coatings are shown by reference char-

acters 15 and 16 in FIGURES 1 and 2, 31 in FIGURE 3, and 41 in FIGURE 4.

A method which is quite generally applicable to abrasives of the type described utilizes the desired metal or indeed mixture of metals as a metal-leaf pigment in a vehicle, such as a varnish or lacquer base. The metal-leaf pigment is applied in such a way that it is adherent to the abrasive particles, which may readily be accomplished by including a small amount of a suitable binding agent with the metal-leaf pigment. In general, formulations for aluminum varnish or bronze-leaf varnish and similar coatings generally may be used. For simplicity in presentation, it will be understood that when an adherent layer of a metal-leaf pigment is mentioned herein, particularly in the claims, it is to be understood that sufficient of a suitable binding agent, such as a varnish or lacquer vehicle, is present in the formulation to cause adherence of the metal-leaf pigment to the surfaces so treated, and coherence of the pigment particles to each other. The metal-leaf pigment may be combined with the so-called size coats, that is, the adhesive coatings applied to the abrasive granules after they have been embedded in the maker coat, or the metal-leaf pigment may be applied as a separate coating after the size coat or coats have been applied, or it may even replace the size coat or coats themselves.

All of the metals which are commonly and generally employed in surface coatings of this type, wherein the metal is formed into a metal-leaf pigment and dispersed in a suitable coating or suspending vehicle, may be used. Aluminum and the various brasses, known in the metal-leaf pigment art as "bronzes," stainless-steel leaf pigments, and nickel leaf pigments are available and suitable. Such metal-leaf pigments are most commonly made by comminuting the desired metal, as by spray atomizing in the molten condition, followed by ball-milling so that the individual metal particles are flattened out into a flake or leaf form; or they may be produced by a stamping process. Some fatty organic material such as stearic acid or tallow is commonly used not only to assist in the ball-milling process but also to enhance the leafing action when mixed with the vehicle.

Of the metal-leaf pigments available, the aluminum and copper leaf pigments are generally pure aluminum and pure copper respectively. Stainless steel leaf pigment is generally 18-8 chromium-nickel alloy. The copper-zinc alloys contain from 10 to 35% zinc, while the copper-zinc-aluminum alloys contain up to 15% each of zinc and aluminum in addition to the copper.

In the practice of my invention I do not confine myself to the use of a single metal or alloy in a particular application; I have found that various mixtures of these are specially suitable in the practice of my invention. For example, the following mixtures can be used, the figures denoting parts by weight in the different lettered mixtures:

| Metal of the Leaf Pigment | A | B | C | D | E | F | G | H | I |
|---------------------------|---|---|---|---|---|---|---|---|---|
| Aluminum-----             | 1 |   | 1 | 1 | 1 | 1 |   | 1 |   |
| Copper-----               | 2 | 1 | 1 | 1 |   | 1 | 1 |   | 1 |
| Copper-zinc-----          |   | 1 |   |   |   | 1 |   | 1 |   |
| Copper-zinc-aluminum----- |   | 1 |   |   |   |   | 1 |   |   |
| Stainless steel-----      | 1 | 1 | 1 | 2 |   |   | 1 | 1 | 1 |
| Nickel-----               |   |   |   |   |   |   |   |   | 1 |

The thickness of the individual flakes of such pigments is exceedingly small, being generally as low as  $\frac{1}{20,000}$  of an inch. The other dimensions are of course generally larger, and the metal-leaf pigments are available in a considerable range of particle sizes. For my purposes I choose metal-leaf pigment particles considerably smaller in all dimensions than the granules of abrasive to be coated. This is readily done since the average metal-leaf pigment particle is substantially smaller than the average abrasive particle size, and for abrasive granules of small

particle size it is merely necessary to use a particularly fine metal-leaf pigment. The reason that this is done is so that the metal-leaf pigment coating may readily conform to the surface of the abrasive granule or particle and form a coating which is thin relative to the particle size. A thickness of the adherent layer, containing the metal-leaf pigment particles,  $\frac{1}{2}$  to  $\frac{1}{200}$  the average abrasive particle diameter will be found particularly suitable, although I do not mean to limit myself in this respect.

It will of course be understood that when a layer of metal-leaf pigment particles is laid down in the fashion described, because of the extreme thinness of the individual flaky metal particles there will be a number of particles comprising the thickness of the layer. Accordingly, when a metal-leaf pigment layer is recited in this specification and in the claims which follow, it will be understood that this refers to a layer made up of a multiplicity of overlapping metal flakes, in which the layer itself is a number of times the thickness of the individual flakes.

Where an abrasive article of the coated type is to be processed in accordance with the invention, using a metal-leaf pigment, the varnish or lacquer metal-leaf pigment formulation can be applied by usual and known means such as application by brush, spraying, dipping, roll-coating, and the like. Where metal-leaf pigment is to be applied to a coherent mass of granules as is the case with a grinding wheel, then the grinding wheel may be dipped in the suspension containing the metal-leaf pigment. Where the average pore space in the abrasive article is large, simple dipping suffices for considerable penetration and coating of the walls of the pores within the mass of abrasive particles. However, this action is facilitated by utilizing pressure to force the metal particles into the abrasive article. For example, where a number of grinding wheels are to be treated, they are placed in a pressure container and covered with metal-leaf pigment formulation, whereupon pressure is applied to the container, thus forcing the liquid containing the metal-leaf pigment into the pores. Upon release of pressure, much of the liquid will be forced out again by air compressed within the pores, but this will still leave an adherent metallic coating on the particles. The excess liquid may be removed from the grinding wheels by centrifugal force. Drying or setting of the remainder takes place as usual.

Extensive tests have proved the peculiar and unexpected advantages arising from the metal-leaf pigment coating as described in accordance with the present invention. Examination of both coated abrasive and coherent granular abrasive articles such as grinding wheels and abrasive blocks which have been treated in accordance with the invention show some wholly unexpected and valuable phenomena. In the first place, the individual abrasive granules tend to wear down more gradually and cleanly and only on their outermost projections, that is, on the portions of the granules actually exposed to the work-piece. The metal-leaf pigment layer prepared in accordance with the invention remains intact, even under conditions of severe use. Of course, as an individual abrasive granule gradually wears away, the metal-leaf pigment coating wears along with it, but not to any appreciable extent below the height of the actual working abrasive surface. This situation is shown in FIGURES 2 and 3, where the truncated tops of the abrasive particles shown are the result of use of the abrasive article in actual grinding work.

The mechanism of the abrading away of abrasive granules in actual use is not fully known, but it is believed by some workers to consist of a series of microscopic chipping actions. Without desiring to be held to any theory of action, I believe that the longer life of abrasives made in accordance with the present invention may at least in part be ascribed to the control over this chipping action which is brought about by the presence of the metal-leaf pigment layer. This layer will tend to prevent gross chipping away of an abrasive granule, by the pro-

tection which it offers to the sides of the granule below the working face.

In some cases it appears that a portion of the metal-leaf pigment layer migrates to the truncated tops of the partially abraded or chipped abrasive granules while the abrasive article is in use, and this film, while exceedingly thin, nevertheless performs some useful functions, such as that of a solid lubricant. This action continues during the useful life of the abrasive article.

While I do not wish to be limited to any theory of action, it seems clear, after studying the results obtained in practical tests, that the metal-leaf pigment layer performs at least two functions which bear directly on the superior results obtained. In the first place, the metal-leaf pigment layer, remaining as it does intact up to the actual cutting edges of the particles, and having an extremely high metal content, serves as an excellent heat conductor and substantially reduces the temperature obtained at the cutting edges of the granules while in use. While the metal-leaf pigment layer is thin, the distances involved are short, and since it is ever so much better a conductor of heat than the materials of the commonly used abrasive granules, bonds and sizing, the enhanced cooling action is appreciable.

Another important role played by the metal-leaf pigment layer is to form a heavy-duty solid lubricant for the sides and even the cutting edges of the particles. This is especially so when the metal of which the pigment is composed is relatively soft and ductile, as is the case for example with aluminum, aluminum alloys, copper, and copper alloys; but lubrication is still appreciable in the case of nickel and stainless steel metal-leaf pigments, which doubtless arise from the small particle size and the flaky character of the particles. This lubricating action is important in preventing undesired seizure of the abrasive particles, whereby they might otherwise be dislodged or prematurely chipped away. Because of the flat nature of the metal-leaf pigment particles, considerable orientation of the flakes parallel to the adjacent abrasive particle surface takes place. In actual use the metal-leaf pigment layer tends to become burnished or polished, thus lowering even more the coefficient of friction to the workpiece as well as the grinding debris which ordinarily collects in the interstices between the abrasive granules. A startling effect produced in abrasive articles made in accordance with the invention is the almost complete elimination of any tendency for the abrasive article to "block up" or "glaze," that is, to retain the grinding debris in the abrasive article instead of allowing it to be carried away by the various forces operating during grinding. This again is a consequence of the lubricating action of the metal-leaf pigment layer, as well as its smooth surface, and heat conducting properties.

The action of metal-leaf pigments appears to be unique in this regard, for the covering of the abrasive particles by various mineral pigments, such as the various lead, zinc, and titanium oxides and silicates, zinc and barium sulphates and carbonates, and calcium carbonates and silicates, as used in paints, for example, does not lead to this desirable effect at all, and indeed worsens matters. While again I do not wish to be bound to any one theory of action, it appears that this stems from the fact that mineral paint pigments of this type lack both the solid-lubricant property and the good heat conductivity discussed above.

In some cases, when dealing with coated abrasives, it will be found advantageous to apply a metal-leaf pigment coating of the type described to the back side of the backing, as well as to the front side which contains the abrasive granules. This is shown in section in FIGURE 4, wherein 40 is an adherent metal-leaf pigment layer on the back of a coated abrasive article. This is a convenient means of reducing friction on the backing and of reinforcing it, and furthermore encloses the entire coated abrasive article within an imperious sheath. When

the backside of the backing is so coated as has been described, another advantage accrues in better conduction of heat away from the actual portions of the abrasive article which are in grinding service at the time. Shelf life of the article is also increased in this manner.

Some working examples will now be given.

*Example 1*

An aluminum oxide grinding wheel, vitrified bond, eight inches in diameter by one inch thick, with a  $\frac{5}{8}$  inch center arbor opening, composed of size 30 abrasive grain, meeting U.S. Department of Defense MIL-STD-165, page 15, and designated A 30H9V in accordance with the terminology of U.S. Military Specification MIL-W-16714A, was immersed for a period of five minutes in a mixture 15 of the following ingredients, and prepared in the following proportions: two pounds of aluminum metal-leaf pigment conforming to Federal Specification TT-A-468a, Type I, Class B, per one gallon of varnish conforming to Federal Specification TT-V-109, and three pints of mineral spirits conforming to TT-T-291a, Grade 1. Upon removal from the suspension the excess material was spun off by centrifugal force, and the remaining layer was then allowed to dry. Grinding tests on a variety of soft, medium, and hard steels, using an untreated wheel 25 of otherwise like specification as a control, disclosed several advantages derived from the application of the metal-leaf pigment layer, viz., a substantially reduced rate of wear, improved grinding action, including better finishes on the steels dealt with, and the substantially complete elimination of any tendency to accumulate or retain grinding debris within the pores of the wheel.

*Example 2*

An endless abrasive belt, 4" x  $37\frac{1}{2}$ ", composed of silicon carbide cloth, said material conforming to Federal Specification P-C-451-A, Type II, Class I, and the abrasive having a grit number of 100 as defined in paragraph 3.5.2 of said specification; and a cloth backed abrasive disc, ten inches in diameter and with no center hole, coated on one side with aluminum oxide having a grit number of 50 as above defined, these materials also conforming to the foregoing specification, and designated as Type I, Class I, therein; were spray-coated on their abrasive side with a fluid mixture consisting of two pounds of bronze-flake pigment conforming to Federal Specification TT-P-340, in the only grade recognized by this specification; per one pound of aluminum metal-leaf pigment, one gallon of varnish, and two and one-half pints of mineral spirits, each as used and described in Example 1. The two articles were allowed to dry, and were then mounted on a combination belt-disc sander. In control tests made, a second belt and disc of duplicate specifications, but not containing the metal-leaf pigment surface layer, was used as a standard of comparison. The materials surfaced consisted of various metals and woods ranging from medium to hard to very hard, and the tests included treatment of flat surfaces, curves, angles and edges of the various woods and metals. The treated belt and disc showed a number of improved properties, including increased durability, performance, and economy. Better finished surfaces were evident, increased ease of operation was noted, and less evidence of wear, loading, and glazing was observed.

*Example 3*

Aluminum oxide coated-abrasive paper sheets, 9" x 11", some having a grit number of 60, and others having a grit number of 120, the abrasive and the grit sizes conforming to P-C-451-A, Type I, of Example 2, were roll-coated with a copper-zinc bronze metal-leaf pigmented vehicle blend, prepared in the proportions of three pounds of bronze pigment as described in Example 2, to one gallon of mixing varnish conforming to Federal Specification TT-V-119, and one quart of turpentine. After dry-

10

15

20

25

30

35

40

45

50

55

60

65

70

75

ing, one sheet of each grit size was cut into three equal size strips of three and two-thirds inches by nine inches each, to fit a vibratory sanding machine, and four 5" discs, two of each grit size, were cut from two other sheets, for use on a portable power sander, using a conventional resilient back-up pad. All were used for sanding, variously, rock maple, white oak, yellow pine, and fillings of automobile body solder contained in a repair on a sheet steel automobile fender, as well as adjoining portions of the fender itself. In all cases the abrading action was more effective than with similar strips and discs which had not been coated. The usual tendency for abrasive articles of this type to "fill-in" between the abrasive particles with the material being abraded was substantially reduced, producing faster and cleaner abrading action, increased tear resistance, and extended the serviceability of the treated abrasive strips and discs.

*Example 4*

An aluminum oxide wheel (disc) twelve inches in diameter, resinoid bond, comprised of size 46 abrasive grain, corresponding to the specification of Example 1, relating to abrasive wheels, and constructed with means for attachment to a steel machine-face-plate used on general purpose horizontal disc grinders wherein the grinding takes place on the flat side of the wheel rather than on the outside edge as distinguished from a grinding wheel, was immersed in a fluid mixture conforming to the following proportions of ingredients; one gallon of the varnish vehicle of Example 3, one pound of the aluminum metal-leaf pigment of Example 1, one pound of copper-zinc bronze metal-leaf pigment of Example 2, and one pound of 325 mesh stainless steel metal-flake pigment of 18-8 chromium-nickel steel, plus one-half gallon of xylene. The disc was kept submerged in the mixture for a period of two minutes, during which time a pressure of 40 pounds per square inch was applied, thereafter, the disc was removed, the excess fluid mixture thereon was spun off by centrifugal force, and the remainder permitted to dry. Tests were then made on carbon steel, alloy steel, and on hard cast bronze, with results markedly superior to those of the untreated control disc of otherwise like specification, in abrasive durability and grinding efficiency.

*Example 5*

Three garnet coated abrasive sanding discs, nine inches in diameter and having no center hole, cut from three garnet paper sheets conforming to Federal Specification P-P-121a, Class 1, with a grit number of 1/0-80 as defined in paragraph 3.1.7 of said specification, were brush-coated on their abrasive surfaces with a metal-leaf pigment layer made up of the following combination of ingredients and proportions, for application thereto: two pounds of aluminum metal-leaf pigment as used and defined in Example 1, per one gallon of varnish vehicle conforming to Federal Specification TT-V-81b, Type II, Class A, cut with three pints of mineral spirits as used and defined in said Example 1. The articles were permitted to air dry for a period of 48 hours, after which time they were affixed adhesively, one at a time, to a metal sanding plate for use on a power disc sander. Tests were made using pine, fir, and cedar. In all three cases, marked superiority was shown over the three control sanding discs, cut from like garnet sheets but minus the metal-leaf pigment coating. This was evidenced from the standpoint of durability and overall rate of wear of the inventive articles over relatively long periods of use. Substantially reduced was the normal tendency to "fill-up" with particles of the material being sanded, thus eliminating to a considerable extent the usual and objectionable inclination to glaze, snag, and tear, excessively or prematurely.

*Example 6*

An aluminum oxide coated abrasive belt, 6" x 48", having a grit number of 40, conforming to the specifica-

tion of Example 2, relating to belts, was roll-coated on the underside, that is the cloth side, as well as on the abrasive surface, with the metal-leaf pigment-varnish mixture used and described in Example 1. The rate of wear of the belt during grinding tests made, working steel, cast bronze, and cast alloy aluminum, was found to be appreciably lower than was a similar belt to which the backing layer had not been applied. In addition, freer, cleaner, and cooler cutting was also observed, especially, the work done at the arc areas of contact, at either extremity, where belt and drum are in immediate and continuous contact, and where heat is most easily generated in a belt sanding procedure.

*Example 7*

Flint-coated abrasive paper sheets equivalent to Federal Specification P-P-105, Class 1, and Class 2, with grit designations of Fine (F), Medium (M), and Coarse (C), as defined in Table III, page 3, of said specification, were first spray-coated with a fluid mixture prepared in the following proportions: per three pounds of the stainless steel metal-flake of Example 4, one gallon of the varnish vehicle and one quart of the solvent-thinner of Example 5. This was followed by a spray application of the aluminum metal-leaf pigment mixture of said Example 5, and the sheets were then allowed to air-dry. When tests were made, using untreated flint abrasive paper sheets of the same specification as controls, on sawed wood, primed wood, painted wood, and fiberboard, employing hand work, as well as a portable power sander using discs cut from the abrasive papers, and also, with the power sander on shoe sole leather, substantial increases in abrasive life and cutting quality were observed, as were decreases in loading and glazing.

*Example 8*

A silicon carbide grinding wheel, vitrified bond, eight inches in diameter, having a face thickness of one inch, and a  $\frac{5}{8}$  inch center arbor opening, composed of abrasive grain size 60, meeting U.S. Department of Defense MIL-STD. 165, page 15, and designated C60G8V in accordance therewith, was immersed in a fluid consisting of a heat resistant silicone resin varnish vehicle, pigmented with two pounds of aluminum metal-leaf pigment particles per one gallon of vehicle, conforming to U.S. Military Specification MIL-P-14276 (Ord), and diluted with two-thirds gallon of toluene. The wheel was allowed to remain submerged for a period of two minutes, during which time a pressure of 50 pounds per square inch was applied. It was then removed from the mixture, the excess fluid immediately spun off by centrifugal force, and the remaining residue was allowed to dry. Thereafter, grinding tests on low tensile strength materials including cast iron, unannealed malleable iron, 18-8 stainless steel, aluminum, brass, marble, ceramics, and glass, were made using an untreated wheel of otherwise like specification as a control. The treated wheel performed in a superior manner as regards freer and cleaner grinding, durability, and over-all efficiency, including finer resultant surfaces.

The best method of practicing the invention of which I am aware is the use of aluminum metal-leaf pigment of the type described, and in a varnish vehicle of the type described, both as in Example 8 hereinabove, applied to a silicon carbide grinding wheel. However, the application of my invention for example to coated abrasives as set forth in Example 2 shares fully in the advantages of the invention, so that Example 2 may be termed nearly the best mode as well.

As has been explained hereinabove, this invention is broadly applicable to particles of an abrasive substance which are held in fixed relationship to one another, such as for example by being bonded to a cloth, paper or metal backing, or by being bonded in the mass as in a grinding wheel. This is broadly distinguished from a slurry of a powdered abrasive material in a liquid such as water, as

is used in certain types of metal grinding, in stone cutting, and the like. As used herein and in the claims which follow, accordingly, the term "abrasive article of manufacture" includes all such articles of the type described wherein the particles of abrasive granules are fixed with relation to each other by the various means described. The invention obviously is not applicable to a slurry of freely mobile abrasive particles forming part of a liquid slurry, and by the same token such a slurry is not an "abrasive article of manufacture" either in common parlance, or in the terminology of the art, and of this specification and of the claims appended hereto.

Having described the invention, I claim:

1. An abrasive article of manufacture, comprising, a plurality of granules of an abrasive substance, portions of said granules being exposed and other portions of said granules being attached to a bonding material, said exposed portions of said granules and exposed portions of said bonding material being coated with an adherent layer of a metal-leaf pigment.
2. The article of manufacture of claim 1 in which the metal is aluminum.
3. The article of manufacture of claim 1 in which the metal is copper.
4. The article of manufacture of claim 1 in which the metal is a copper-zinc alloy.
5. The article of manufacture of claim 1 in which the metal is a copper-zinc-aluminum alloy.
6. The article of manufacture of claim 1 in which the metal is stainless steel.
7. An abrasive article of manufacture, comprising, a plurality of granules of an abrasive substance, portions of said granules being exposed and other portions of said granules being attached to a bonding material, said exposed portions of said granules and exposed portions of said bonding material being coated with an adherent layer of a metal-leaf pigment, said layer being a thickness of about  $\frac{1}{2}$  to about  $\frac{1}{200}$  of that of the diameter of said granules.
8. A coated abrasive, comprising, a sheet backing, a plurality of granules of an abrasive substance bonded to said backing with a bonding material, said granules and said bonding material being coated with an adherent layer of a metal-leaf pigment.
9. The coated abrasive of claim 8 in which the metal is aluminum.
10. The coated abrasive of claim 8 in which the metal is copper.
11. The coated abrasive of claim 8 in which the metal is a copper-zinc alloy.
12. The coated abrasive of claim 8 in which the metal is a copper-zinc-aluminum alloy.
13. The coated abrasive of claim 8 in which the metal is stainless steel.
14. The coated abrasive of claim 8 in which the layer has a thickness of about  $\frac{1}{2}$  to about  $\frac{1}{200}$  of that of the diameter of said granules.
15. A coated abrasive, comprising, a sheet backing having a front side and a back side, a plurality of granules of an abrasive substance bonded to the front side of said backing with a bonding material, said granules and said bonding material and said back side being coated with an adherent layer of a metal-leaf pigment.
16. The coated abrasive of claim 15 in which the metal is aluminum.
17. The coated abrasive of claim 15 in which the metal is copper.
18. The coated abrasive of claim 15 in which the metal is a copper-zinc alloy.
19. The coated abrasive of claim 15 in which the metal is a copper-zinc-aluminum alloy.
20. The coated abrasive of claim 15 in which the metal is stainless steel.
21. An abrasive article of manufacture, comprising, a coherent mass of granules of an abrasive substance, said

granules being bonded at their points of contact with a bonding material and presenting open spaces between said granules whereby portions of said granules and portions of said bonding materials are exposed, said exposed portions of said granules and said exposed portions of said bonding material being coated with an adherent layer of a metal-leaf pigment.

22. The abrasive article of claim 21 in which the layer has a thickness of about  $\frac{1}{2}$  to about  $\frac{1}{200}$  of that of the diameter of said granules.

23. The abrasive article of claim 21 in which the metal is aluminum.

24. The abrasive article of claim 21 in which the metal is copper.

25. The abrasive article of claim 21 in which the metal is a copper-zinc alloy.

26. The abrasive article of claim 21 in which the metal is a copper-zinc-aluminum alloy.

27. The abrasive article of claim 21 in which the metal is stainless steel.

28. An abrasive article of manufacture, comprising, a plurality of granules of an abrasive substance, portions of said granules being exposed and other portions of said granules being attached to a bonding material, said exposed portions of said granules and exposed portions of said bonding material being coated with an adherent layer of a metal-leaf pigment chosen from the group consisting of aluminum, copper, copper-zinc alloy, copper-zinc-aluminum alloy, nickel, and stainless steel and mixtures thereof.

29. The method of treating an abrasive article of manufacture of the type which consists essentially of a coherent mass of granules of an abrasive substance and in which the granules are bonded at their points of contact with a bonding material and present open spaces between the granules whereby portions of said granules and portions of said bonding materials are exposed, which includes the steps of: immersing the said article of manufacture in a suspension of a metal-leaf pigment in a set-

5

10

15

20

25

30

table fluid adhesive vehicle, applying pressure thereto so as to force the suspension into the said open spaces, releasing said pressure, removing said article of manufacture, permitting said article of manufacture to drain off excess suspension, and allowing the so treated article to stand until said suspension remaining in said article has set.

30. The method in accordance with claim 29 in which the settable fluid adhesive vehicle is chosen from the class consisting of varnishes and lacquers.

31. An abrasive article of manufacture, comprising a plurality of granules of an abrasive substance chosen from the class consisting of flint, garnet, alumina, silicon carbide, glass, quartz, diamond, and mixtures thereof: portions of said granules being exposed and other portions of said granules being attached to a bonding material chosen from the class consisting of hide glue, starch glue, varnish, shellac, alkyd resins, phenolic resins, polyester adhesives, natural rubber adhesives, synthetic rubber adhesives, sodium silicate, and ceramic bodies; said exposed portions of said granules and exposed portions of said bonding material being coated with an adherent layer of metal-leaf pigment chosen from the class consisting of aluminum, aluminum-beryllium alloy, copper, copper-zinc alloy, copper-lead alloy, copper-zinc-lead alloy, beryllium copper, stainless steel, nickel, gold, silver, and platinum and mixtures thereof.

## References Cited in the file of this patent

## UNITED STATES PATENTS

|           |                |       |                |
|-----------|----------------|-------|----------------|
| 2,050,992 | Aust           | ----- | Aug. 11, 1936  |
| 2,353,404 | Keeleric       | ----- | July 11, 1944  |
| 2,368,473 | Keeleric       | ----- | Jan. 30, 1945  |
| 2,374,331 | Cooke          | ----- | Apr. 24, 1945  |
| 2,542,058 | Riedesel       | ----- | Feb. 20, 1951  |
| 2,853,401 | Mackiw et al.  | ----- | Sept. 23, 1958 |
| 2,906,612 | Anthony et al. | ----- | Sept. 29, 1959 |
| 3,031,344 | Sher et al.    | ----- | Apr. 24, 1962  |